

# United States Patent Office

2,921,027

Patented Jan. 12, 1960

1

2,921,927

## ANTI-RUST LUBRICATING OIL

Elmer W. Brennan, Carpentersville, Ill., assignor to The Pure Oil Company, Chicago, Ill., a corporation of Ohio

No Drawing. Application July 26, 1957  
Serial No. 674,300

9 Claims. (Cl. 252—32.7)

This invention relates to improved anti-rust lubricating oils and, more particularly, to lubricating oil compositions which pass the U.S. Navy static water-drop corrosion test designated as MIL-P-17272 (SHIPS), dated July 18, 1952. This test will hereinafter be referred to as the static water drop corrosion test.

This application is a continuation-in-part of application Serial Number 420,435, filed April 1, 1954, now abandoned, by the present inventor.

The problem of protecting metallic equipment from atmospheric corrosion is one of long standing. A particularly acute problem is that of protecting internal combustion engines and other equipment exposed to the severely corrosive atmosphere encountered in coastal areas or on ship board and in many industrial areas. The internal combustion engines used in military equipment are often subjected to long periods of storage or exposure to corrosive environments during transportation and must be protected. During operation these engines are often exposed to corrosive atmospheres and the exhaust gases therefrom, especially from spark-ignition engines, produce corrosive atmospheres which deleteriously affect metal parts with which they come in contact. Under emergency situations, sea water is sometimes used as a coolant in these engines and every effort must be made to protect the metal parts as long as possible.

Many techniques and compositions have been proposed to protect metal surfaces from corrosion, i.e., by the use of removable protective coatings known as slushing compounds or rust-preventive compositions classified as oils and greases. Most of these compositions are intended for use in the metallic equipment during periods of storage as in gun barrels and breeches, metal containers, machinery in idle status, finished machine parts in storage, and emergency equipment used during wartime or in stock piles. For these purposes the compositions are generally screened by means of the well-known humidity

cabinet test conducted for 200 hours at 100° F. and 100 percent humidity with fresh saturated air being supplied at a rate between 1 and 1.5 complete changes per hour. Also, the hydrobromic acid tests are used to measure the ability of rust-preventive lubricants to neutralize acidic corrosive atmospheres, particularly the acidic products present in exhaust gases. It has been found that known rust inhibitors which function to transform lubricating oils into rust-preventive lubricants for use under these storage conditions fail to provide the type of protection necessary to pass the static water drop corrosion test.

This invention is based on the discovery of a new property of a class of compounds known as "Tweens" by the Atlas Powder Company, that is, the ability of this type of compound to carry lubricating oil compositions through the critical static water-drop corrosion test and thereby meet the requirements for a rust inhibitor for crankcase lubricating oils, specifically Class A, Navy 9000 series crankcase lubricants. "Tweens" are polyoxyethylene sorbitan esters of fatty acids. A specific product known as "Tween 81" has the following general characteristics:

|    | Property                          | Value          |
|----|-----------------------------------|----------------|
| 25 | Hydrophile-Lipophile Balance..... | 10.0.          |
|    | Form at 25° C.....                | oily liquid 1. |
|    | Viscosity (cp. at 25° C.).....    | 350-550.       |
|    | Specific gravity.....             | 1.00-1.05.     |
|    | Flash Point (° F.).....           | 550.           |
|    | Fire Point (° F.).....            | 600.           |
| 30 | Color.....                        | lemon.         |

<sup>1</sup> Tends to gel on standing.

"Tween 81" is a non-ionic surface-active agent. The property of hydrophile-lipophile balance is an empirical number assigned by The Atlas Powder Company to their surface-active agents to represent the relative oil or water affinity of the material. An agent having a hydrophile-lipophile balance of about 2.0 to 9.0 is classifiable as 35 lipophilic (oil-living). An agent having a hydrophile-lipophile balance of 15.0-18.0 is designated as hydrophilic (water-living). "Tween 81" is intermediate in regard 40 this property. As to the solubility at 25° C. in various agents, the following information is available: "Tween 81" is dispersible in distilled water, hard water, 5% 45  $H_2SO_4$ , 5%  $NaOH$ ,  $Na_2SO_4$ , and 5%  $AlCl_3$ . In non-aqueous solvents, "Tween 81" is generally soluble or dispersible, requiring, in some instances, the use of high concentrations or careful adjustment of the concentration.

50 Reactions showing the preparation of "Tweens" may be represented as follows:



where  $R$  is the residue of a long-chain fatty acid such as oleic, lauric, palmitic or stearic,  $N = n_1 + n_2 + n_3$  and indicates the number of moles of ethylene oxide and  $n_1$ ,  $n_2$  and  $n_3$  are any whole numbers from 1 to 7, inclusive.

In "Tween 81" RCOOH is oleic acid, N has a value of 3 to 6, and accordingly,  $n_1$ ,  $n_2$  and  $n_3$  have values of 1 to 4 and may be the same or different. One skilled in the art will know that the anhydrierization of sorbitol in the above reaction is shown to involve the hydrogen attached to the first carbon atom and the hydroxyl group on the 5th carbon atom. This reaction, as is known, may involve the hydrogen of the first carbon atom of the sorbitol molecule and the hydroxyl group of the fourth carbon atom in which event an ether ring having five carbon atoms results and the subsequent reaction with fatty acid and ethylene oxide results in a product having the following formula:

(II)



( $n_1$ ,  $n_2$  and  $n_3$  having the values aforementioned and R being a fatty acid residue).

Compounds of both Formula I and Formula II are contemplated by this invention and in fact are present as a complex mixture in the product known as "Tween 81." Increases in the amounts of ethylene oxide used in the reaction to the point where N has a value of 7 to 20 results in a product known as "Tween 80" which for purposes of this invention is equivalent to "Tween 81," being also polyoxyethylene sorbitan monoleate. "Tween 80" has the same corrosion-inhibiting properties as "Tween 81" as far as the purposes of this invention are concerned. These products are generally used to form emulsions, their respective abilities in this regard, as measured by the interfacial surface tensions in dynes at 25° C., being equivalent at concentrations of 0.1 weight percent and varying at lesser and greater concentrations. "Tween 80" has an HLB factor of 15.0 and is an oily liquid, having a viscosity (cp. at 25° C.) of 350-550, a sp. gr. of 1.06-1.10, flash point 605° F., fire point of 645° F. and is a lemon-yellow color. The chemical name of polyoxyethylene sorbitan monoleate will be used in the balance of the specification and claims to mean either or both "Tween 80" and "Tween 81" and mixtures of same having either a 4 carbon atoms ether ring, or a 5 carbon atom ether ring, or both, as indicated heretofore. Although the invention will be demonstrated by reference to experiments using "Tween 81" the invention will apply to polyoxyethylene sorbitan fatty esters broadly, regardless of the number of ethylene oxide groups reacted with each molecule of the ether-ester.

Accordingly, a primary object of this invention is to provide a lubricating composition which meets the requirements of the static water-drop corrosion test MIL-P-17272 (SHIPS), July 18, 1952.

Another object of the invention is to provide a lubricating composition which meets the engine performance requirements of M.S. 9030 oil (MIL-L-9000A), and also the static water-drop test, by including in said composition a minor proportion of polyoxyethylene sorbitan ester of a fatty acid, particularly the monoleate ester.

Other objects and advantages of the invention will become apparent as the description thereof proceeds.

To demonstrate the invention, a number of known rust inhibitors were tested in a base mineral oil composition fortified with a detergent-inhibitor and a commercial corrosion inhibitor. The base or blank oil consisted of:

92.0 weight percent intermediate V.I. oil (200 vis. neutral).

5.4 weight percent of a detergent inhibitor consisting of a mixture of 3.44 weight percent mineral lubricating oil, 1.35 wt. percent of barium diisobutyl phenol sulfide and 0.61 wt. percent of calcium petroleum sulfonate.

2.6 weight percent zinc hexyl dithiophosphate.

This base mineral oil composition so fortified meets the U.S. Navy engine performance requirements of M.S. 9030 oil (MIL-L-9000A) using a GM 71 engine. The zinc hexyl dithiophosphate is a commercial corrosion inhibitor which in itself or in combination with the detergent-inhibitor does not pass the static water-drop corrosion test, but is used to meet the other anti-corrosion properties necessary to qualify the base composition to meet the M.S. 9030 oil requirements, which tests include bearing corrosion tests, etc. These addends are subsequently further defined.

The results of these experiments are set forth in the following table wherein blend No. 1 is the base oil just described.

TABLE I  
*Static water drop corrosion test*

| No. | Additive                           | Conc. In<br>Percent | Time for<br>Rust<br>Formation       |
|-----|------------------------------------|---------------------|-------------------------------------|
| 1   | Blank                              |                     | 24 hours.                           |
| 2   | Zinc naphthenate                   | 0.15                | 48 hours.                           |
| 3   | do                                 | 0.075               | Do.                                 |
| 4   | Proprietary inhibitor A            | 0.04                | Do.                                 |
| 5   | Proprietary inhibitor B            | 0.08                | Do.                                 |
| 6   | Barium petroleum sulfonate         | 0.10                | 12 hours.                           |
| 7   | do                                 | 0.20                | Do.                                 |
| 8   | do                                 | 0.30                | Do.                                 |
| 9   | Organic phosphate                  | 0.10                | Stain at 48<br>hours <sup>1</sup> . |
| 10  | Barium petroleum sulfonate         | 0.20                | 48 hours.                           |
| 11  | do                                 | 0.40                | Do.                                 |
| 12  | Sorbitan monoleate                 | 0.25                | Do.                                 |
| 13  | Glycerol monoleate                 | 0.25                | Do.                                 |
| 14  | Polyoxyethylene sorbitan monoleate | 0.25                | Stain at 96<br>hours <sup>2</sup> . |

\* Specimen was stained with surface disturbed.

Specimen was stained with no surface disturbances.

An M.S. 9030 oil should show no rust at the end of 96 hours' testing. In addition, an M.S. 9030 oil must have a viscosity at 210° F. of 58 to 70 SUS, a flash point of about 390° F. minimum, and a maximum pour point of about 10° F. The procedure in MIL-P-17272 (SHIPS), July 18, 1952, comprises subjecting a  $\frac{1}{32}$ -inch-thick, cold-rolled, steel sheet (SAE 1020) specimen shaped as an equilateral triangle to dimpling at its center to a depth of 0.110 inch. The dimple side is thoroughly polished with fine sand paper, and cleaned with C.P. benzene and petroleum ether. After cleaning, the specimen is quickly immersed in the oil sample with the concave side of the dimple uppermost. The container containing the test oil and specimen is then placed in an oven at  $140 \pm 2$ ° F. for one hour. After this, the container and contents are removed from the oven and a drop of water (0.2 ml.) is placed in the oil so as to rest in the shallow depression or dimple in the steel specimen by using a clean hypodermic syringe. The container is then covered with a glass cover, stored in the oven at  $140 \pm 2$ ° F., and observed daily for signs of failure, that is, the first sign of rust which definitely increases in intensity on the next day.

65 From the table it is seen that the oil alone showed  
rusting at the end of 24 hours and certain of the addends  
actually accelerated the rusting. The composition of in-  
hibitor A is not available. All of these products includ-  
ing barium petroleum sulfonate, the organic phosphate,  
70 etc. are well-known corrosion inhibitors. Only poly-  
oxyethylene sorbitan monolates meet the requirements  
of the static water-drop test.

Broadly, this invention relates to the discovery that polyoxyethylene sorbitan esters of fatty acids have the ability to carry a mineral lubricating oil, whether fort-  
76

fied by other addends or not, through the static water-drop corrosion test. The preferred compounds for this purpose are the monoleate esters which are known as "Tween 80" and "Tween 81," the latter compound being used to demonstrate the invention by blend No. 14.

The amount of the sorbitan derivatives used may vary somewhat within the prescribed limits depending on the overall composition and the oxidation-detergent or other addends present therein. In general, about 0.2 to 0.40 weight percent of polyoxyethylene sorbitan monoleate has been found to satisfactorily carry the composition through this severe rust test. About 0.2 weight percent is the minimum that will give assured protection and quantities over about 0.40 do not show any detectable decrease in the degree of staining.

The oil compositions intended by this invention may include other addends such as thickeners, V.I. improvers, oiliness agents, pour-point depressants, other anti-oxidants and other well-known types of addends, or may comprise a mineral lubricating oil and the polyoxyethylene sorbitan monoleates alone in the amounts specified. Although this invention is limited to compositions passing the static water-drop corrosion test designated as MIL-P-17272 (SHIPS), it is not limited to the type of oil used in the experiments. Any mineral lubricating oil may be used whether obtained from Mid-Continent, Pennsylvania Coastal, or Texas crudes. The lubricating oil may be a light or heavy oil of the solvent-refined or conventionally-refined variety. The invention should be distinguished from the prior art which shows the use of sorbitan monoleate as a corrosion inhibitor in oils by means of the humidity cabinet test, or other tests using a corrosive atmosphere of a haloacid, since there is no relationship or correlation between compositions which pass the cabinet test and the problem confronting one in relation to the critical static water-drop corrosion test, a particularly difficult species of corrosion test. Other specific examples of compositions of this invention are set forth in the following table:

TABLE II

| Blend No.                                     | Constituent | Composition (Wt. percent) |      |       |       |
|-----------------------------------------------|-------------|---------------------------|------|-------|-------|
|                                               |             | 15                        | 16   | 14    | 17    |
| Mineral lubricating oil (200 vols. Neutral)   |             | 91.8                      | 91.6 | 91.77 | 91.81 |
| Detergent-inhibitor consisting of:            |             |                           |      |       |       |
| (1) Mineral lubricating oil                   |             | 3.44                      | 3.44 | 3.43  | 3.43  |
| (2) Ba Salt of diisobutyl phenol sulfide      |             | 1.35                      | 1.35 | 1.35  | 1.36  |
| (3) Calcium sulfonate                         |             | 0.61                      | 0.61 | .60   | .60   |
| Zinc hexyl dithiophosphate                    |             | 2.6                       | 2.6  | 2.59  | 2.59  |
| Polyoxyethylene sorbitan monoleate (Tween 81) |             | 0.2                       | 0.4  | 0.24  | 0.21  |

The detergent-inhibitor used in the compositions of this invention are described in United States Patent 2,379,241 by McNab and U.S. Patent 2,761,845 by Rogers. Broadly, this addend may comprise an oil-soluble metal salt having the general formula,



where M is a metal, preferably a divalent metal, cobalt, barium, calcium, aluminum, zinc, magnesium, cadmium, tin, lead, chromium, manganese and nickel; Y is a member of the right-hand side of group VI of the periodic table of elements, as oxygen or a member of the sulfur family; Ar is an aromatic nucleus such as benzene, or a condensed ring nucleus such as naphthalene, anthracene, etc.; Z is sulfur, selenium or tellurium; x is an integer of from 1 to 5, preferably 1 or 2; Q is an organic group which may be identical with the part of the compound which is on the left side of Z, or a group having a somewhat similar type of structure, or it may be a hydrocarbon group such as amyl, octadecyl, or aralkyl as

benzyl, or aryl as tolyl; and  $R_m$  represents one or more hydrocarbon groups such as alkyl, or alkenyl, e.g., amyl, octyl, octenyl, etc., or cyclo-aliphatic, e.g., cyclohexyl. Examples are the cobalt or barium salts of hydroxy

5 tertiary-amyl phenyl sulfide, and the cobalt or barium salts of hydroxy diisobutyl phenyl sulfide. In place of the calcium petroleum sulfonate, any oil-soluble metal salt of an acidic organic compound may be used, i.e., the mixed aluminum-calcium soap of acids obtained in the oxidation of sweater oil, or nickel oleate. In general, from about 0.01 to 6.5 weight percent of the finished addend containing about 63.75 wt. percent of a mineral lubricating oil, 25.0% of the barium salt and about 11.25% of the calcium petroleum sulfonate is used. A 10 species of this addend sold under the trade name of Paranox 65, has the following properties:

Typical physical characteristics:

|                                 |      |
|---------------------------------|------|
| Viscosity @ 210° F., SSU        | 130  |
| Flash point, °F.                | 425  |
| Pour point, °F.                 | 10   |
| Specific gravity, 60/60° F.     | 1.02 |
| Weight, avg., lb./gal. @ 60° F. | 8.5  |

Typical chemical characteristics:

|                               |           |
|-------------------------------|-----------|
| Barium, wt. percent           | 7.9       |
| Calcium, wt. percent          | 0.6       |
| Sulfur, wt. percent           | 2.7       |
| Ash, wt. percent              | 14.9      |
| Sulfated ash, wt. percent     | 15.8      |
| Conradson carbon, wt. percent | 16.7      |
| Neutralization No., ASTM      | 9 (basic) |

The zinc hexyl dithiophosphate may be replaced with other commercial addends designed for this purpose, such as zinc or cadmium alkyl dithiophosphates including zinc 35 heptyl dithiophosphate, cadmium heptyl dithiophosphate, zinc octyl dithiophosphate, cadmium octyl dithiophosphate, etc.

What is claimed is:

1. A lubricating oil composition consisting essentially 40 of a major portion of a mineral lubricating oil, a small amount of a polyvalent metal salt of an alkyl phenol sulfide selected from the group consisting of the barium salt of diisobutyl phenol sulfide, the cobalt salt of diisobutyl phenol sulfide, the barium salt of tertiary amyl phenol sulfide, and the cobalt salt of tertiary amyl phenol sulfide, a small amount of calcium petroleum sulfonate, a small amount of a polyvalent metal salt of an alkyl dithiophosphate selected from the group consisting of zinc hexyl dithiophosphate, zinc heptyl dithiophosphate, zinc octyl dithiophosphate, cadmium heptyl dithiophosphate, and cadmium octyl dithiophosphate, and at least about 0.2 weight percent of a polyoxyethylene sorbitan mono-fatty acid ester containing from 3 to 6 moles of ethylene oxide per molecule wherein the fatty acid esterifying 45 group is selected from the group consisting of oleate, laurate, palmitate and stearate groups.

2. A lubricating composition in accordance with claim 1 in which said polyvalent metal salt of an alkyl phenol sulfide is the barium salt of diisobutyl phenol sulfide.

3. A lubricating composition in accordance with claim 1 in which said polyvalent metal salt of an alkyl dithiophosphate is zinc hexyl dithiophosphate.

4. A lubricating composition in accordance with claim 1 in which said polyoxyethylene sorbitan mono-fatty acid 65 ester is polyoxyethylene sorbitan monoleate.

5. A lubricating oil composition characterized by its ability to meet the requirements of an M.S. 9030 oil and pass the static water-drop corrosion test designated as MIL-P-17272-SHIPS, consisting essentially of about 91 70 weight percent of a mineral lubricating oil, about 5.4 weight percent of a detergent-inhibitor consisting of the following:

(1) About 3.44 weight percent of a mineral lubricating oil carrier.

(2) About 1.35 weight percent of a phenol sulfide salt selected from the group consisting of the barium salt of diisobutyl phenol sulfide, the cobalt salt of diisobutyl phenol sulfide, the barium salt of tertiary amyl phenol sulfide, and the cobalt salt of tertiary amyl phenol sulfide and

(3) About 0.61 weight percent of calcium petroleum sulfonate,

about 2.6 weight percent of an alkyl dithiophosphate salt selected from the group consisting of zinc hexyl dithiophosphate, zinc heptyl dithiophosphate, zinc octyl dithiophosphate, cadmium heptyl dithiophosphate, and cadmium octyl dithiophosphate and between about 0.2 and 0.4 weight percent of polyoxyethylene sorbitan mono-fatty acid ester containing from 3 to 6 moles of ethylene oxide per molecule wherein the fatty acid portion is selected from the group of oleate, laurate, palmitate and stearate groups.

6. A lubricating composition in accordance with claim 5 in which said phenol sulfide salt is the barium salt of diisobutyl phenol sulfide.

7. A lubricating composition in accordance with claim 5 in which said alkyl dithiophosphate salt is zinc hexyl dithiophosphate.

8. A lubricating composition in accordance with claim 5 in which said polyoxyethylene sorbitan mono-fatty acid ester is polyoxyethylene sorbitan monoleate.

9. A lubricating oil composition, characterized by its ability to meet the requirements of an M.S. 9030 oil and pass the static water-drop corrosion test designated as MIL-P-17272-SHIPS, comprising about 91 weight percent of a mineral lubricating oil, about 5.4 weight percent of a detergent-inhibitor consisting of about 3.44 weight percent of a mineral lubricating oil, about 1.35 weight percent of the barium salt of diisobutyl phenol sulfide and 0.61 weight percent of calcium petroleum sulfonate, about 2.6 weight percent of zinc hexyl dithiophosphate and between about 0.2 to 0.4 weight percent of polyoxyethylene sorbitan monoleate containing from 3 to 6 moles of ethylene oxide per molecule.

15

References Cited in the file of this patent

UNITED STATES PATENTS

|           |                |               |
|-----------|----------------|---------------|
| 2,470,537 | Waugh          | May 17, 1949  |
| 2,479,424 | Sproule et al. | Aug. 16, 1949 |
| 2,560,202 | Zimmer et al.  | July 10, 1951 |
| 2,565,403 | Sproule et al. | Aug. 21, 1951 |

OTHER REFERENCES

25 "Atlas Surface Active Agents," Atlas Powder Co., Wilm., Del., 1948; Table I (facing page 26) and page 29.